

## UNITED STATES PATENT OFFICE.

THEODORE H. KOHLER, OF BLOOMFIELD, NEW JERSEY, ASSIGNOR TO THE OCEAN LEATHER CO., INC., OF NEW YORK, N. Y., A CORPORATION OF DELAWARE.

## DEARMORED LEATHER.

No Drawing.

Application filed July 23, 1921. Serial No. 487,211.

*To all whom it may concern:*

Be it known that I, THEODORE H. KOHLER, a citizen of the United States, and residing at Bloomfield, in the county of Essex and 5 State of New Jersey, have invented a new and Improved Dearmored Leather, of which the following specification is a full disclosure.

This invention relates to tanned fish-skins, 10 and is in the nature of an article of manufacture characterized by its complete freedom superficially as well as subcutaneously, from the dermal armor or papillæ-scabrous material constituting the protective 15 layer of a skin of a shark or the like.

A shark-skin has never been produced entirely free from its dermal armor; especially in a thoroughly tanned condition. Many attempts have been made to produce such 20 a leather, but they have all failed completely to get rid of its so-called "shagreen" by reason of the fact that it is composed of a myriad of papillæ-scabrous teeth projections, each of which has its root firmly em- 25 bedded in minute sockets in the epidermis of the skin. These papillæ have always resisted any attempts to remove them by purely mechanical means, such as through the use of abrasive wheels, or scraping implements. 30 While the protruding portions may be more or less completely worn away, their roots will remain irremovable in the pores or sockets, and it has therefore been impossible to produce a satisfactory piece of leather 35 from such skins. Likewise, all attempts to remove the "shagreen" through the agency 40 of chemicals have had the effect of destroying the corium of the skin; making it im- 45 possible to produce a satisfactory piece of 50 leather.

I have nevertheless succeeded in producing a completely de-armed sharp-skin in a thoroughly tanned condition and with the epidermal surface substantially intact; the 45 pores of the resultant leather being freed from the papillæ so that its epidermal sur- 55 face possesses a flexibility substantially equal to the finest grades of leather pro- 60 duced from other sources. This epidermal 65 surface after treatment is very tough com- 70 pared to ordinary leather and is highly re- 75 sistant to abrasion, barking, or scuffing. My 80 product furthermore is uniformly absorp- 85 tive to various conventional dye-stuffs so 90 that it admits being colored as easily, as 95

freely and as perfectly as any other species of leather. Also, it is tough to an extraordinary degree and yet can be cut or sewed without difficulty in contradistinction from shark-skins which contain in their pores 60 the stumps of the papillæ.

My new product may easily be made by means of the process disclosed in my co-pending application for Letters Patent of the United States Serial Number 487,210 65 filed July 23, 1921.

Briefly stated, the process used by me for the preparation of my new species of leather is based upon the discovery that if the raw skin be first converted into leather by means 70 of a vegetable tanning process, the papillæ will not be rendered resistant to the action of the hydrochloric acid; whereas the true skin will not be affected. The hydrochloric acid will render the papillæ sufficiently sol- 75 uble or at least so far loosen their bondage that they may be easily removed together with the sub-surface portions thereof by the application of water accompanied by some mechanical attrition, such as scouring 80 or tumbling. The treatment is preferably effected as follows:

In carrying out my process as I prefer to employ it, the raw skin—that is, the skin after removal from the fish and with the 85 armor thereon,—should be thoroughly tanned before removing the shagreen, and preferably by means of suitable organic tanning agents, such for example as the vegetable tanning extracts of quebracho, hemlock, sumac, oak, gambier, etc. The tanning methods set forth in the United States Patents Nos. 1,230,266, June 19, 1917, and 1,256,974, Feb. 19, 1918 to Kristian Bendixen, may be resorted to except in so far as they refer 90 to the use of chrome tanning materials. It is important that the tanning be thoroughly accomplished, and I have found that vegetable or other organic agents preferably 95 should be employed. After the tanning it 100 will be found that the flintlike nodules of the armor have been loosened from their adhesions in the pores or depressions in the skin, and may be easily removed as a whole without leaving roots in the pores. I have 105 discovered that the effect of this tanning agent is to convert the raw skin into a true leather displaying a high resistance to an agent capable of acting on the papillæ which, for some reason, are not rendered re- 110

sistant thereto in the course of the specified tanning process. The de-armoring agent to be employed should be one of such a nature that it will metamorphose untanned, or 5 insufficiently tanned, material in the nature of skin.

The next step may be effected advantageously by putting the tanned skins into a tumbling barrel containing a solution of hydrochloric acid in the proportion of from 10 twenty-two to twenty-four gallons of HCl (at 18 Bé.) to about five hundred pounds of skin. The rotation is continued for two to three hours, with the result that the papillæ 15 are loosened and disintegrated and are, by the attrition, separated from the hide, and they may be washed away as minute nodules. Then washing is effected for about an hour by continuing the rotation; using 20 water. Thereby, the acid is eliminated; the final washing being accomplished preferably by means of a solution of borax (say one pound of borax for each two hundred pounds 25 of hide) and any residual acid is thereby neutralized.

The hides from the tumbling barrel will be found quite free from any armor and will be perfectly tanned and nowise injured by the treatment, but in a condition to undergo 30 any suitable finishing processes. For example, they now will readily and uniformly accept the coloring material conveniently employed for finished leather and, after the coloring has been done, they may 35 be oiled and dried and are thus made ready for the market.

The resultant leather displays a handsome grained surface entirely devoid of its original armor and is tough and tenacious to 40 an extraordinary degree and may be readily cut, sewed, embossed and otherwise worked up into various articles of manufacture. The epidermal surface is in its natural condition, retaining all the wear and abrasive- 45 resistant qualities which the leather should have in its final form.

As an alternative to the above-mentioned continuous scale-removing steps, it is quite feasible to apply the acid by hand to the 50 previously-tanned hides for painting a succession of coats of acid on the armored side at intervals of about six hours until the papillæ have become sufficiently disintegrated or loosened from the epidermis to permit 55 them to be eliminated by the action of water and a scraping implement. It has

been found that the acid mentioned has the effect of rendering the papillæ more or less soluble in water, preferably by converting them into gelatine so that their removal 60 becomes a simple matter.

The above mentioned process is not claimed herein; but is made the subject matter of my other application for patent; this application being directed to the product as an article of manufacture.

I therefore claim as new and desire to secure by Letters Patent:

1. Leather consisting of the tanned skin of an armored fish, freed of the armor including the sub-surface portions, but retaining in substance the natural epidermal surface. 70

2. Leather consisting of tanned skin of an armored fish, freed of the armor including the sub-surface portions but containing the 75 depressions from which the armor has been removed and retaining in substance the natural epidermal surface.

3. Tanned shark skin leather from which the armor has been completely removed and 80 the outer surface of which has a toughness greater than that of the underlying leather body, and comprising substantially the whole epidermal skin.

4. Leather comprising the tanned skin of a shark with the armored portion thereof substantially completely removed, but leaving the natural epidermal surface substantially intact and having a multiplicity of raised portions on said epidermal surface of greater resistance and wear than the main body portion of said leather, whereby the 85 said surface is rendered relatively non-scuffing. 90

5. Leather consisting of skin of an armored fish tanned by an organic tanning material, and which has been freed of the armor including the sub-surface portions, but retaining in substance the natural epidermal surface. 95

6. Leather consisting of the tanned skin of an armored fish, freed of the armor including the sub-surface portions and having a regularly grained epidermal surface which is substantially non-scuffing. 100 105

In witness whereof, I hereunto subscribe my name, as attested by the two subscribing witnesses.

THEODORE H. KOHLER.

Witnesses:

H. S. DOTTENHER,  
MARTHA GROSSMAN.